

Sept. 4, 1923.

1,466,837

E. KARDOS

TIN SPONGE ARTICLE OF MANUFACTURE AND METHOD OF PRODUCING AND  
UTILIZING THE SAME  
Filed Dec. 27, 1919



INVENTOR

*Emanuel Kardos*  
BY  
*Chas. F. Dane*  
HIS ATTORNEY

## UNITED STATES PATENT OFFICE.

EMANUEL KARDOS, OF NEWARK, NEW JERSEY, ASSIGNOR TO METAL & THERMIT CORPORATION, OF CHROME, NEW JERSEY, A CORPORATION OF NEW JERSEY.

TIN SPONGE ARTICLE OF MANUFACTURE AND METHOD OF PRODUCING AND UTILIZING THE SAME.

Application filed December 27, 1919. Serial No. 347,753.

*To all whom it may concern:*

Be it known that I, EMANUEL KARDOS, a citizen of Hungary, and resident of Newark, in the county of Essex and State of New Jersey, have invented certain new and useful Tin Sponge Articles of Manufacture and Methods of Producing and Utilizing the Same, of which the following is a specification.

10 The invention relates to the protection of tin sponge against the effects of oxidation, and to this end comprises a novel article of manufacture and the method of producing and utilizing the same, by coating or impregnating tin sponge with chloride of zinc, and, preferably compressing the tin sponge so treated into briquette form, and ultimately recovering the tin in solid form and substantial purity by melting the admixture at a temperature approximating the melting point of the tin and below the boiling point of the zinc chloride, and finally separately withdrawing the molten tin and zinc chloride.

25 In the past the operation of melting tin sponge has been difficult, expensive and wasteful of tin, because of the large surface which the sponge offers to contact with the air, which results in rapid oxidation of the tin even when the sponge has been hydraulically compressed. In fact, in order to melt the sponge without serious loss due to oxidation, it has been found necessary to effect the melting operation under conditions of total exclusion of air, and usually with the employment of reducing agents such as carbon and the like, which is effective to reduce any tin oxide which may be formed or which may be present. This latter operation, however, can be carried out successfully only at a high temperature, and with the concurrent formation of slag, which is unavoidable, so that the entire operation results in a large loss of tin, due 45 partly to the metal being entrapped in the slag, and partly to the volatilization of the metal and the carrying away of the fumes by the draft necessary to produce the required high temperature.

50 According to the present invention all of the objections and difficulties aforesaid are eliminated and it is possible to prepare the tin sponge so that the same may be kept indefinitely without danger of impair-

ment by oxidation or deterioration, and when it is desired to recover the tin in merchantable form the composite body of tin sponge and impregnating zinc chloride may be readily melted at a relatively low temperature, without the formation of slag and without substantial loss of metallic tin. These results are obtained by applying zinc chloride, preferably in solution, to tin sponge, in sufficient quantity to cause the zinc chloride to substantially envelop and cover the exposed surfaces of the sponge, and preferably to impregnate the porous body of the sponge, thereby excluding air or other reagents which would tend to deleteriously affect the tin. This coating or impregnating of the porous tin sponge with zinc chloride may be effected in various ways, as by dipping the sponge in a solution of the chloride, spraying the sponge with the solution, or by mixing and agitating the sponge and the solution in a suitable receptacle until the solution permeates the sponge and covers the surfaces of the latter. Preferably the impregnated or coated sponge is compressed into briquettes of suitable size which facilitates the handling and storage of individual bodies of sponge and also removes any excessive liquid. When it is desired to recover the tin and also the impregnating zinc chloride the bodies or briquettes of impregnated tin sponge are placed in a suitable vessel, preferably an open steel kettle, and heated to a temperature of approximately 230° C. at which temperature both the tin and the chloride of zinc melts. The chloride of zinc, being of lower specific gravity than the tin, will float on top of the molten tin and protect the latter completely against the oxidizing effect of the air. The water associated with the zinc chloride will evaporate, but the chloride of zinc will be left intact provided the temperature is not raised above the boiling point of the salt, viz: 262° C. After the first batch has been melted the impregnated briquettes or bodies of tin sponge and chloride of zinc may be added from time to time, and as the briquettes or bodies have a lower specific weight than metallic tin but a higher one than the zinc chloride they will be entirely submerged in the molten zinc chloride and thus be protected against any oxidizing effect. The

zinc chloride may be ladled off or otherwise withdrawn from time to time in a fused state and may be used again for treating further quantities of tin sponge, and any metal particles of tin entrapped in the same may be subsequently recovered. Likewise the molten tin may be withdrawn by any suitable means and allowed to cool, preferably under conditions which will reduce superficial oxidation to a minimum.

A simple and effective form of apparatus for carrying out the operation aforesaid is illustrated in the accompanying drawing, in which A represents a metallic kettle or receptacle having an overflow spout C. Centrally mounted within the kettle A and passing through the cover thereof, is a metallic cylinder B provided with an overflow spout D, said cylinder being preferably open at the bottom and provided with lateral peripheral orifices to allow the molten metal to flow into the kettle A. The upper portion of the cylinder B is provided with splash plates E', E'', and with a thermometer F which dips into the molten zinc chloride and affords a ready check on the temperature of the molten bath. The apparatus as described may be fired by gas, oil or any other suitable means which is capable of ready regulation to maintain the desired temperature, slightly in excess of that required to melt the tin, as hereinbefore described.

The tin sponge coated or impregnated with chloride of zinc, and preferably in briquette form, is charged into the cylinder B through the opening in the top thereof between the splash plates E', E'', and heat applied to the kettle A sufficient to melt the tin, but below the boiling point of zinc chloride. The molten tin sinks to the bottom of the cylinder B and then passes out into the kettle A where it accumulates until it overflows at spout C. The molten zinc chloride, however, being of lighter specific gravity than the molten tin, floats on the latter and is retained in the cylinder B, as indicated, so that when additional quantities of impregnated tin sponge are charged into the apparatus through the top of cylinder B they are completely submerged in the molten zinc chloride. As indicated, as the molten zinc chloride accumulates the excess overflows the entrance of spout D and is discharged from the apparatus. The principal object of treating the tin sponge with zinc chloride is to prevent oxidation of the metallic sponge before and during the process of melting, but especially be-

fore the melting operation begins and also to permit the tin sponge treated with the zinc chloride to be stored for any length of time without impairment of the metallic tin, as by oxidation, which would quickly destroy the sponge if the same were untreated in the manner specified. Furthermore, the tin sponge thus treated can be readily melted at a relatively low temperature without material loss of the metal, without the formation of slag or the use of reducing agents, and with a substantially complete recovery of the metallic tin as well as the impregnating zinc chloride.

What I claim is:

1. The method of protecting tin sponge which comprises coating the same with chloride of zinc.

2. The method of protecting tin sponge which comprises impregnating and coating the same with a solution of chloride of zinc.

3. The method of protecting tin sponge against oxidation during the melting of the same which consists in impregnating the sponge with chloride of zinc, and heating the same to a temperature below the boiling point of the chloride of zinc.

4. The method of protecting tin sponge against oxidation during the melting of the same which consists in impregnating the sponge with chloride of zinc, compressing the mixture into briquettes, and heating the briquettes in a suitable vessel to a temperature approximating that of the melting point of the tin.

5. The method of protecting tin sponge against oxidation during the melting of the same which consists in impregnating the sponge with chloride of zinc, compressing the mixture into briquettes, heating the briquettes in a suitable vessel to a temperature approximating that of the melting point of the tin, and separately withdrawing the molten tin and zinc chloride.

6. An article of manufacture comprising a body of tin sponge coated with chloride of zinc.

7. An article of manufacture comprising a compressed body of tin sponge coated with chloride of zinc.

8. An article of manufacture comprising an admixture of tin sponge and chloride of zinc compressed into briquette form.

Signed at Chrome in the county of Middlesex and State of New Jersey this 18th day of December A. D. 1919.

EMANUEL KARDOS.